



US005679118A

## United States Patent [19]

Jarvis et al.

[11] Patent Number: 5,679,118

[45] Date of Patent: Oct. 21, 1997

## [54] REFINING PROCESS AND APPARATUS

[75] Inventors: David A. Jarvis, Coral Springs, Fla.; Ewert J. A. Wilson, Albany, Ky.

[73] Assignee: Research Octane Inc., Albany, Ky.; a part interest

[21] Appl. No.: 735,931

[22] Filed: Oct. 23, 1996

## Related U.S. Application Data

[63] Continuation-in-part of Ser. No. 605,282, Feb. 8, 1996, abandoned, which is a continuation-in-part of Ser. No. 430,275, Apr. 28, 1995, abandoned, which is a continuation-in-part of Ser. No. 385,466, Feb. 8, 1995, abandoned.

[51] Int. Cl. 6 C10L 1/18

[52] U.S. Cl. 44/451

[58] Field of Search 44/451; 585/1

## [56] References Cited

## U.S. PATENT DOCUMENTS

|           |         |               |
|-----------|---------|---------------|
| 1,858,822 | 5/1932  | Frolich       |
| 1,878,170 | 9/1932  | Naiman et al. |
| 2,012,199 | 8/1935  | McElroy       |
| 2,365,009 | 12/1944 | Robertson     |
| 4,243,493 | 1/1981  | Gruber et al. |
| 4,296,262 | 10/1981 | Grane et al.  |
| 4,296,263 | 10/1981 | Worrell       |
| 4,297,172 | 10/1981 | Kyle          |

|           |         |                |         |
|-----------|---------|----------------|---------|
| 4,304,948 | 12/1981 | Vora et al.    | 585/315 |
| 4,393,259 | 7/1983  | Ward et al.    | 585/315 |
| 4,403,999 | 9/1983  | Bezman         | 44/56   |
| 4,444,988 | 4/1984  | Capsuto et al. | 585/415 |
| 5,017,731 | 5/1991  | Gesser et al.  | 568/910 |
| 5,093,533 | 3/1992  | Wilson         | 585/1   |
| 5,171,912 | 12/1992 | Harandi        | 585/301 |
| 5,310,954 | 5/1994  | Hiles et al.   | 549/429 |
| 5,348,707 | 9/1994  | Harandi et al. | 44/449  |

Primary Examiner—Jacqueline V. Howard  
Attorney, Agent, or Firm—Oltman, Flynn & Kubler

## [57] ABSTRACT

A process of producing high octane alcohols includes the steps of preparing a first mixture of substantially ethanol and butane or natural gasoline, the mixture having a certain temperature and a certain pressure, adjusting the certain pressure of the mixture to a magnitude within the range of 10 to 50 pounds per square inch, adjusting the temperature of the mixture to a magnitude within the range of 100 to 350 degrees Fahrenheit, adjusting the pressure of the mixture to a pressure within the range of 500 to 1000 pounds per square inch, catalyzing the mixture with a platinum catalyst, lowering the temperature of the mixture to a magnitude within a range of 90 to 190 degrees Fahrenheit, and separating out liquid product and gas from the mixture. Then a second mixture of said liquid product and methanol is prepared and the process steps are repeated on this second mixture to produce a second product plus gas.

3 Claims, 1 Drawing Sheet





FIG. 1



FIG. 2

## REFINING PROCESS AND APPARATUS

## RELATED APPLICATIONS

This application is a continuation-in-part of application Ser. No. 08/605,282 filed Feb. 8, 1996, now abandoned, which is a continuation-in-part of application Ser. No. 08/430,275 filed Apr. 28, 1995 (now abandoned), which in turn is a continuation-in-part of application Ser. No. 08/385,466 filed Feb. 8, 1995, (now abandoned).

## FIELD OF THE INVENTION

The present invention relates generally to the field of fuel forming processes. More specifically it relates to a process of producing high octane alcohols, including the steps of placing a pre-mixed mixture of ethanol and butane or natural gasoline in a starting tank, raising the pressure of gases above the surface of the mixture to fifty pounds per square inch, pumping the mixture from the bottom of the starting tank through a first high pressure conduit into a heat exchanger where the temperature of the mixture is raised to a magnitude within the range of 100 to 350 degrees Fahrenheit, extracting the heated mixture from the heat exchanger with high pressure pumps which raise the mixture pressure to 500 to 1000 pounds per square inch, and feeding the heated and pressurized mixture through a seconds high pressure conduit through a nozzle and through a third high pressure conduit into an elongate catalyzing chamber containing a platinum catalyst. Additional steps include delivering the catalyzed mixture through a fourth high pressure conduit into a cooler for lowering the temperature to a magnitude within a range of 90 to 190 degrees Fahrenheit feeding the cooled mixture through a fifth high pressure conduit into a series of separator tanks in which liquid final product collects in the tank bottoms and gas rises within the tanks above the surface of the liquid, and the liquid is drained off as the final product. The final product is 120 to 160 research octane, 110 to 129 motor octane, R & M about 148.

## BACKGROUND OF THE INVENTION

There have long been various chemical processes for producing gasoline and other fuels. A problem with these prior processes has been that they either fail to produce high octane gasoline, or they fail to do so efficiently.

These prior processes include that of Harandi, U.S. Pat. No. 5,171,912, issued on Dec. 15, 1992. Harandi discloses a process for the production of C<sub>6</sub>-gasoline from n-butane and propane. The Harandi process includes the steps of contacting a fresh feedstream including normal butane with shape selective medium pore zeolite catalyst particles under conditions sufficient to convert n-butane to an effluent stream including C<sub>6</sub>-alkanes; separating the effluent stream in a fractionator to recover an overhead stream including propane; contacting the propane stream and a fresh propane feedstream with shape selective, medium pore zeolite catalyst particles under conversion conditions sufficient to convert propane to a mixture including C<sub>6</sub>-alkanes; deethanizing the mixture and passing the deethanized product including C<sub>6</sub>-alkanes to the fractionator for separation concurrent with the effluent stream; recovering a bottom stream including C<sub>6</sub>-gasoline from the fractionator; preferably, distilling an intermediate stream including C<sub>6</sub> alkanes from the fractionator and recovering a stream including isobutane and a stream including unconverted normal butane; and recycling the unconverted normal butane to the normal butane feedstream to the integrated process.

Ward, et al., U.S. Pat. No. 4,393,259, issued on Jul. 12, 1983, reveals a process for converting propane or butane to gasoline. The Ward, et al. process includes the steps of passing feed hydrocarbon into a dehydrogenation zone; passing the entire dehydrogenation zone effluent including hydrogen and light by-products into a catalytic condensation zone where the resulting olefins are converted into dimers and trimers; passing the condensation zone effluent stream into a separation zone in which the dimers and trimers are concentrated into a product stream, with unconverted feed hydrocarbon and hydrogen being recycled to the dehydrogenation zone.

Vora, et al., U.S. Pat. No. 4,304,948, issued on Dec. 8, 1981, teaches a multi-step hydrocarbon conversion process for converting butane to gasoline. The process includes the steps of passing butane into a dehydrogenation zone and the entire dehydrogenation zone effluent is then passed into a catalytic condensation zone where butylene is converted into C<sub>6</sub> and C<sub>7</sub> hydrocarbons; commingling and separating the condensation zone effluent, a stripper overhead stream and an absorber bottoms stream into vapor and liquid portions; passing the liquid into the stripper and contacting the vapor portion with stripper bottoms liquid in an absorber; contacting the absorber overhead stream with liquid butane in a second absorber to remove C<sub>6</sub> hydrocarbons and recycling the dehydrogenation zone; and debutanizing a portion of the stripper bottoms to yield the liquid butane and a gasoline product.

Capsuto, et al., U.S. Pat. No. 4,444,988, issued on Apr. 24, 1984, discloses the use of liquefied propane and butane or butane recycled to control the heat of reaction of converting olefins to gasoline and distillate. The Capsuto, et al. process uses beds and separates the effluent product from the beds into a gas in a liquid phase, cools the gas phase to form additional liquid and heat exchanges the liquid with the overhead gas from the separator.

Wilson, U.S. Pat. No. 5,093,533, issued on Mar. 3, 1992, reveals blended gasolines and a process for making the blended gasolines. The Wilson process involves mixing of a butane-pentane rich component, and natural gasoline component, and at least one octane-enhancing component. The mix is weathered during the blending operation to remove light-weight hydrocarbons including two, three and four-carbon components.

Hiles, et al., U.S. Pat. No. 5,310,954, issued on May 10, 1994, discloses a process for preparing tetrahydrofuran. The Hiles et al. process separates tetrahydrofuran from a feed mixture containing water, lower alkanol and tetrahydrofuran, which includes distilling the mixture in a first distillation zone at a first pressure; recovering from an upper part of the distillation zone a first vaporous mixture including water, lower alkanol and tetrahydrofuran; subjecting the material from the first vaporous mixture to condensation conditions in a condensation zone; passing condensate from the condensation zone to a second distillation zone operated at a second pressure higher than the first pressure; recovering from an upper part of the second distillation zone a second vaporous mixture including water, lower alkanol and tetrahydrofuran that has a lower concentration of tetrahydrofuran than the first vaporous mixture; and recovering from a lower part of the second distillation zone a stream including substantially pure tetrahydrofuran.

It is thus an object of the present invention to provide a process of producing a very high octane alcohol product efficiently.

It is another object of the present invention to provide such a process which can be practiced with conventional heat exchanger and separator tank equipment.

It is still another object of the present invention to provide such a process which is safe to practice.

It is finally an object of the present invention to provide such a process which is inexpensive to practice.

### SUMMARY OF THE INVENTION

The present invention accomplishes the above-stated objectives, as well as others, as may be determined by a fair reading and interpretation of the entire specification.

A process of producing high octane alcohols is provided, including the steps of preparing a mixture of substantially ethanol and butane or natural gasoline, the mixture having a certain temperature and a certain pressure, adjusting the certain pressure of the mixture to a magnitude within the range of 10 to 50 pounds per square inch, adjusting the temperature of the mixture to a magnitude within the range of 100 to 350 degrees Fahrenheit, adjusting the pressure of the mixture to a pressure within the range of 500 to 1000 pounds per square inch, catalyzing the mixture with a platinum catalyst, lowering the temperature of the mixture to a magnitude within a range of 90 to 190 degrees Fahrenheit, and separating out liquid product and gas from the mixture. The process preferably includes the additional steps of delivering a quantity of the gas separated from the liquid product into a furnace to supply heat required for the process, and the further additional steps of delivering a quantity of the gas separated from the liquid product into the mixture at the initial step of the process. The separating step preferably includes several separation steps of separating the mixture into liquid product and gas.

After running the first mixture through the process to produce a liquid product, a second mixture of the liquid product and methanol may be prepared and run through the same series of steps to produce a second product plus gas. The second product typically has an octane rating of 162.8.

An apparatus for producing high octane alcohols is also provided, including a starting tank for retaining a mixture of substantially ethanol and butane or natural gasoline, a heat exchanger for raising the temperature of the mixture, a first high pressure conduit extending from the starting tank to the heat exchanger, a catalyzing chamber, second and third high pressure conduits extending from the heat exchanger to the catalyzing chamber, a nozzle interconnecting the second and third high pressure conduits, high pressure pumps for extracting the heated mixture from the heat exchanger and delivering the mixture to the catalyzing chamber through the second and third high pressure conduits, and a separator for precipitating liquid product out of the mixture.

The catalyzing chamber preferably includes several upright tubular segments, each tubular segment having a top portion and a bottom portion and containing the platinum catalyst, interconnection conduits interconnecting the tubular segments alternatingly across the top and bottom portions of the tubular segments, a baffle plate within at least one of the tubular segments, the baffle plate having several plate ports. The tubular segments each preferably include one baffle plate positioned within and across the top portion and the bottom portion of the tubular segment.

### BRIEF DESCRIPTION OF THE DRAWINGS

Various other objects, advantages and features of the invention will become apparent to those skilled in the art from the following discussion taken in conjunction with the following drawings, in which:

FIG. 1 is a semi-schematic view of the preferred apparatus for carrying out each step of the inventive process.

FIG. 2 is a perspective view of the baffle plate for use in the catalyzing chamber tubular segments.

### DETAILED DESCRIPTION OF THE PREFERRED EMBODIMENTS

As required, detailed embodiments of the present invention are disclosed herein; however, it is to be understood that the disclosed embodiments are merely exemplary of the invention which may be embodied in various forms. Therefore, specific structural and functional details disclosed herein are not to be interpreted as limiting, but merely as a basis for the claims and as a representative basis for teaching one skilled in the art to variously employ the present invention in virtually any appropriately detailed structure.

Reference is now made to the drawings, wherein like characteristics and features of the present invention shown in the various FIGURES are designated by the same reference numerals.

### Process

Referring to FIG. 1, a process of producing high octane alcohols is disclosed, including the following steps. A pre-mixed mixture 10 of one third ethanol and two thirds butane is placed in a starting tank 12. The pressure of gases above the surface of the mixture 10 is raised to fifty pounds per square inch. The mixture 10 is pumped with pumps 14 from the bottom of starting tank 12 through a first high pressure conduit 16 into a heat exchanger 20, where the temperature of mixture 10 is raised to a level within the range of 100 to 350 degrees Fahrenheit. The preferred temperature is 225 degrees Fahrenheit. The heated mixture 10 is extracted from heat exchanger 20 with high pressure pumps 22, which raise mixture 10 pressure to a level within the range of 500 to 1000 pounds per square inch. The preferred pressure is 600 pounds per square inch. The heated and pressurized mixture 10 is fed through a second high pressure conduit 24, through a nozzle 26 and through a third high pressure conduit 32 into an elongate catalyzing chamber 30 containing a platinum catalyst 34. Chamber 30 includes three interconnected upright segments 28. The catalyzed mixture 10 is delivered through a fourth high pressure conduit 42 into a cooler 40 for lowering the mixture 10 temperature to a level within a range of 90 to 190 degrees Fahrenheit.

The cooled mixture 10 is fed through a fifth high pressure conduit 44 into a first separator tank 50 in which final liquid product 60 collects in the bottom of first separator tank 50 and gas 62 rises to fill a space within tank 50 above the surface of liquid product 60. The liquid product 60 is fed through a first separated liquid conduit 72 at the bottom of tank 50 and the gas 62 is drained off through a first separated gas conduit 82 at the top of tank 50. Both liquid product 60 and gas 62 are delivered into a second separator tank 70, in which more liquid product 60 is separated. Some of gas 62 within second separator tank 70 is delivered back through a feedback conduit 100 into the top of starting tank 12. Some of gas 62 within the second separator tank 70 is simultaneously delivered through a second separated gas conduit 84 into a third separator tank 80 where still more liquid product 60 precipitates out and gathers in the bottom of third separator tank 80. Some of gas 62 within third separator tank 80 is drained into a feedback conduit branch 92. Some of gas 62 within third separator tank 80 is delivered through a third separated gas conduit 86 into a furnace 90, where gas 62 is burned as fuel to supply heat to the process where needed.

Final liquid product 60 is within the range of 120 to 160 research octane, 110 to 129 motor octane, and about 148 R and M. Other final product 60 test data are as follows:

|                     |           |           |
|---------------------|-----------|-----------|
| Oxygenates          | L.V. %    | 42.75     |
| MTBE                | L.V. %    | <0.1      |
| TAME                | L.V. %    | <0.1      |
| Alcohols (Ethanols) | L.V. %    | 42.75     |
| <br>G.C. Breakdown  | <br>Wt %  | <br>Vol % |
| N. Butane           | 45.60     | 53.03     |
| ISO ISO Pentane     | 1.42      | 1.55      |
| N. Pentane          | 1.02      | 1.10      |
| Toluene             | 2.02      | 1.57      |
| Ethanol             | 49.94     | 42.75     |
| <br>PONA            | <br>Vol % |           |
| Paraffins           |           | 55.68     |
| Olefins             |           | <0.01     |
| Naphthenes          |           | <0.01     |
| Aromatics           |           | 1.57      |

To produce high octane gasoline, add 20% by volume of the new product to 80 octane gasoline. The resulting mixture is 92.8 octane, with a vapor pressure in the range of 4 to 19 pounds per square inch.

#### Preferred Embodiments of Apparatus

Referring to FIG. 1, a preferred apparatus is disclosed for practicing the above-described process of producing high octane alcohols. This apparatus is merely exemplary and other forms of apparatus are contemplated.

Starting tank 12 is a vertical cylindrical drum. Heat exchanger 20 and pumps 14 and 22 are of any suitable conventional design. Nozzle 26 is preferably about three eights inches diameter. Catalyzing chamber 30 includes three elongate, upright tubular segments 28, each containing platinum catalyst 34. Segments 28 are interconnected by interconnection conduits 110, across the tops of the first and second segments 28 and across the bottoms of second and third segments 28. A baffle plate 120 having a plurality of ports 122 is positioned across the top and bottom of each segment 28. See FIG. 2. Cooler 40 preferably includes a substantially horizontal tray 130 elevated on legs 132. Separator tanks 50, 70 and 80 are vertical cylindrical drums. Tank 70 is preferably of substantially larger diameter than tanks 50 and 80.

Another embodiment of the invention uses as a starting material approximately one third ethanol mixed with two thirds natural gasoline. The process and apparatus for treating this mixture is the same as that previously described and this explanation will not be repeated herein. Natural gasoline is essentially a mixture of butanes and pentanes plus other hydrocarbon materials. Natural gasoline is derived from wet gas by stripping it. An example of natural gasoline is as follows:

C6+ . . . 53.871% by liquid volume  
Butane . . . 3.03% by liquid volume  
Neo-pentane . . . 0.697% by liquid volume  
Iso-pentane . . . 26.046% by liquid volume  
Normal pentane . . . 16.349% by liquid volume.

The resulting product is substantially one half natural gasoline and one half ethanol. It has a vapor pressure of 1.5 to 8.0 psi and an octane rating of 108 to 160.

A further embodiment uses as a starting material a mixture of 10% ethanol and 90% natural gasoline. The process steps and apparatus remain the same. The resulting product showed an increase in octane rating from 72 to 80-100.

It has been found that the starting material may contain 5% to 50% ethanol, and 50% to 95% natural gasoline. It is possible to add to the mixture 3% to 40% butane. The resulting product contains 5-50% ethanol, 50-90% natural gasoline including 3% to 50% hydrocarbons, and a trace of aromatics. The resulting product has a higher octane rating than the starting material. The product has an acceptable vapor pressure. This product appears to be a gasoline grade product. The ethanol can be removed without harming the product.

In the first embodiment, pentane, including iso-pentane, may be substituted for butane in the starting material.

A still further embodiment uses a first mixture consisting of  $\frac{2}{3}$  ethanol and  $\frac{1}{3}$  butane and the process is initially carried out as described in connection with the first embodiment using the same apparatus. The resulting first product has an octane rating of 160. Then another batch consisting of  $\frac{1}{3}$  of the first product and  $\frac{2}{3}$  methanol is run through the same process and apparatus and the resulting second product has an octane rating of 162.8.

While the invention has been described, disclosed, illustrated and shown in various terms or certain embodiments or modifications which it has assumed in practice, the scope of the invention is not intended to be, nor should it be deemed to be, limited thereby and such other modifications or embodiments as may be suggested by the teachings herein are particularly reserved especially as they fall within the breadth and scope of the claims here appended.

We claim:

1. A refining process comprising the steps of:
  - (1) preparing a first mixture of alcohol and butane;
  - (2) adjusting the pressure of said mixture to a magnitude within the range of 10 to 50 pounds per square inch;
  - (3) adjusting the temperature of said mixture to a magnitude within the range of 100 to 350 degrees Fahrenheit;
  - (4) adjusting the pressure of said mixture to a pressure within the range of 500 to 1000 pounds per square inch;
  - (5) catalyzing said mixture with a platinum catalyst;
  - (6) lowering the temperature of said mixture to a magnitude within the range of 90 to 190 degrees Fahrenheit;
  - (7) separating out liquid product and gas from said mixture;
  - (8) preparing a second mixture of said product and methanol, and
  - (9) repeating steps (2) through (7) above on said second mixture to produce a second product plus gas.

2. The refining process of claim 1 in which said first mixture is substantially  $\frac{2}{3}$  ethanol and  $\frac{1}{3}$  butane.

3. The refining process of claim 2 in which said second mixture is substantially  $\frac{1}{3}$  of said first product and  $\frac{2}{3}$  methanol.

\* \* \* \* \*